

## UNITED STATES PATENT OFFICE

2,142,219

## LUBRICANT

Erich M. Steffen, Berlin, Germany, assignor, by  
mesne assignments, of three-fourths to Tide  
Water Associated Oil Company, New York,  
N. Y., a corporation of Delaware

No Drawing. Application August 1, 1933, Serial  
No. 683,169. Renewed September 26, 1938

14 Claims.

(Cl. 87—9)

The present invention relates to improvements in lubricating oils and to certain new compositions of matter, obtained from rubber and the like, which when added to mineral lubricating oils 5 will produce oils of improved qualities.

At the present time most high grade lubricating oils are produced from paraffin or mixed base crude oils. These crude oils contain considerable amounts of waxy materials which have boiling 10 points in the same range as the lubricating oils. In producing lubricating oils two types of stocks are prepared from the crude oil. These stocks are overhead distillates and residual oils, that is, 15 oils which have not been vaporized. Both stocks contain waxy hydrocarbons in amounts sufficient to cause the oil to solidify at moderately high 20 temperatures. Furthermore, wax has no lubricating qualities and will tend to break down at temperatures much lower than the lubricating oil 25 itself. For these reasons it is necessary to remove wax or waxy materials from the oils in order to produce a satisfactory lubricating oil.

In lubricating distillates, the waxy materials are of two distinct types, one of which, on chilling, will separate from the lubricating oil and form relatively large crystals, whereas the other forms small crystals and is known as the amorphous type. It is a relatively simple matter to 30 remove large crystalline waxes by filtration, and this is done in ordinary commercial practice by means of filter presses. In this step the bulk of the wax is removed. However, sufficient wax, predominantly of the amorphous kind, remains in the oil to give high A. S. T. M. pour-points. It 35 is very difficult to remove this type of wax by filtration, since the small crystals do not form rigid and porous filter cakes, in consequence of which the filtration rates are very low. It is possible to remove amorphous wax by filtration, in 40 dilution, with a filter-aid, but again low filtering rates usually make the operation an expensive one.

The concentration of the amorphous wax in such lubricating distillates is low, being approximately 45 2% of the oil, while the crystalline wax may be approximately 10% of the oil. This small amount of amorphous wax is not sufficient to affect the lubricating qualities of the oil. However, at low temperatures sufficient crystals will 50 come out of solution in the oil to give the lubricant an extremely high resistance to flow at low temperatures. This lack of fluidity is indicated by the A. S. T. M. pour-point method. In this test the pour-point is taken as the temperature 55 at which oil will no longer flow when an undis-

tributed body of this oil has been cooled slowly. It can be readily appreciated that in such a test the crystals formed have ample opportunity to grow and interlock, thus forming a relatively rigid structure through the oil. It is generally known that if at the pour-point temperature the crystal structure is broken by stirring, the oil will again flow reasonably freely, indicating that the mere amount of wax present is not sufficient to cause lack of fluidity. Thus, if the amorphous 10 wax on separation can be caused to form still smaller crystals which will not interlock and give this rigid structure at low temperatures, the oil will be a great deal more satisfactory, particularly 15 for use in cold weather in automobiles, for example.

A similar problem in wax removal occurs in the treatment of lubricating oils made from residual oils. Practically all of the waxes contained in such oils are of the amorphous type, and consequently the methods of removal are not by filtration, but settling or centrifuging in solution. It is a relatively easy matter to remove the bulk 20 of the wax, but in order to remove the last traces and insure fluidity at temperatures in the order 25 of 0° to 10° F., exceptionally low separating temperatures are necessary.

I have discovered that the fluidity of wax-containing oils at low temperatures may be insured by the addition of a new composition of matter 30 of great stability, so that this fluidity will be maintained after long periods in storage or after the lubricating oil has been exposed to high temperatures.

In order to prepare this composition of matter, 35 I dissolve a rubber material in a low boiling mineral oil fraction, such as solvent naphtha. A catalyst such as anhydrous aluminum chloride is added at room temperature under agitation and the mixture is kept as these conditions for approximately 16-24 hours. The temperature then is slowly raised to between 140° and 190° F. for about three hours to complete the reaction. The products are allowed to cool and to settle. The sludge is separated and a synthetic product is 45 obtained, dissolved in the solvent mineral oil fraction. After neutralizing the solution by washing with lye and water for example, the synthetic product may be recovered by distilling off the solvent. Additional products may be recovered from 50 the aluminous sludge by admixing the same with water in the presence of a solvent, washing the solution with lye and water and distilling off the solvent.

Rubber materials which I have used for the 55

preparation of these products are crepe rubber, caoutchouc, vulcanized rubber, gutta percha and balata. The products obtained from gutta percha and balata have pour-point depressing properties, though not as pronounced as those of the products made from the other rubbers.

*Example I*

To 15 litres of solvent naphtha, having a boiling range of 200/350° F. is added 680 grams of crepe rubber. The mixture is heated under agitation to 130° F. for three hours and allowed to cool. 200 grams of anhydrous aluminum chloride are slowly added at room temperature and allowed to react for about 16 hours. The temperature is then brought slowly to between 160° and 175° F. and maintained at this point for approximately three hours. Considerable volumes of hydrogen chloride are formed. The final mixture is allowed to cool and the naphtha solution is withdrawn from the sludge. This solution is then purified by washing with an alkaline solution and finally with water. The solution may further be purified by filtration over fuller's earth or similar adsorptive material to improve the demulsibility of the final lubricant, and is finally subjected to distillation for the removal of the solvent naphtha. The synthetic product is obtained as a residue. It has a yellow to red color and proves to have a remarkable stability when brought into contact with concentrated sulphuric acid.

It has the following inspection:

|                                  |          |  |  |
|----------------------------------|----------|--|--|
| Gravity, °A. P. I.....           | 23       |  |  |
| Saybolt viscosity at 100° F..... | 680 sec. |  |  |
| Saybolt viscosity at 210° F..... | 96 sec.  |  |  |

An additional 10 litres of solvent naphtha and 2 litres of water are added to the aluminous sludge and the mixture is agitated for several hours. After settling, the naphtha solution is withdrawn and purified in the manner described above. A distillation residue is obtained as product which has a darker color than the first product and an extremely high viscosity.

The first and the second residual products are then blended with lubricating oil in proportions of 2% by weight of the synthetic product. The A. S. T. M. tests of the original oil and of the blends follow:

| 50 | Tests                            | Original oil | Blended with first product | Blended with second product |
|----|----------------------------------|--------------|----------------------------|-----------------------------|
| 55 | Gravity, °A. P. I.....           | 29.7         | 29.4                       | 29.3                        |
|    | Flash point.....                 | 410° F.      | 410° F.                    | 415° F.                     |
|    | Saybolt viscosity at 100° F..... | 191 sec.     | 189 sec.                   | 208 sec.                    |
|    | Saybolt viscosity at 210° F..... | 47 sec.      | 47 sec.                    | 48 sec.                     |
|    | Pour-point.....                  | +20° F.      | -5° F.                     | -10° F.                     |
| 60 | Color, A. S. T. M.....           | 3 1/4        | 3 1/4                      | 3 1/4                       |
|    | Carbon residue.....              | 0.05%        | 0.04%                      | 0.06%                       |

*Example II*

500 grams of caoutchouc are introduced into 10 litres of naphtha. The mixture is agitated until a homogeneous mixture results. 100 grams of anhydrous aluminum chloride are added at a temperature of about 100° F. The mixture is kept for 3 hours at 120° F. and for additional 2 hours at 170° F. and 2 litres of water are then slowly added. The mixture is finally allowed to cool. The naphtha solution is withdrawn and reduced by fire and steam to about 2 litres. 500 grams of a mineral lubricating oil are added for the purpose of increasing the fluidity of the material, the solution is filtered through a Floridin clay and finally distilled to remove the naphtha.

A residual product is obtained which resembles a very viscous lubricating oil having a viscosity at 210° F. of about 350 Saybolt seconds. The lubricating oil added had a viscosity at 210° F. of 47 Saybolt seconds.

The oil thus obtained was blended with a lubricating oil in proportions of 2% by weight of the synthetic product prepared. The tests of the original oil and of the blend follow:

| 10 | Tests                            | Original oil | Blended with synthetic product |
|----|----------------------------------|--------------|--------------------------------|
| 15 | Gravity, °A. P. I.....           | 29.7         | 29.5                           |
|    | Flash point.....                 | 410° F.      | 410° F.                        |
|    | Saybolt viscosity at 100° F..... | 191 sec.     | 203 sec.                       |
|    | Saybolt viscosity at 210° F..... | 47 sec.      | 48 sec.                        |
| 20 | Pour-point.....                  | +20° F.      | -5° F.                         |
|    | Color, A. S. T. M.....           | 3 1/4        | 3 1/4                          |
|    | Carbon residue.....              | .05          | .04                            |

The examples illustrate that the products described lower the pour-points of lubricating oils to which they are added in small proportions of about 2%.

Depending on the viscosity of the mineral oil with which the rubber conversion products described herein are blended, and the amount of wax therein, amounts of the products up to 5% or even more may be used. For most light and medium motor oils approximately 2% of the product is satisfactory, and for the heavier grades of oil about 3%. Some lowering of pour-point results from addition of the products as low as .05%-1%.

When the products are blended with mineral lubricating oils in proportions larger than about two or three per cent., they have the advantageous effect of reducing the slope of the viscosity-temperature curve of the oil.

The synthetic materials described above may be regarded as isomerization products of rubber materials. As evidenced by their resistance to the action of sulphuric acid, they are highly stable. Such a quality is of extreme value when the products are to be used in motor oils, since the pour-point, as has been found by actual test, will be maintained at or near the original even after the oil has been exposed to high temperature for a considerable length of time.

It is possible to modify the product obtained by manufacturing it in the presence of chlorinated hydrocarbons. In such cases, it is believed that, in addition to the formation of polymerized rubber compounds, a certain lesser amount of condensation of the hydrocarbons on the rubber occurs, and possibly even some polymerization of the chlorinated hydrocarbons themselves. In any event the reactions are extremely complex and products having the same property of reducing pour-points as those described above are obtained, differing only in that their lesser viscosity makes them resemble lubricating oils to a greater extent.

The chlorinated hydrocarbons that are used in the preparation of these modified rubber conversion products may be classed as aliphatic hydrocarbons, though this term is not to be understood as calling for pure aliphatic materials, since mineral oils predominantly aliphatic usually contain some ring compounds.

For this purpose a mineral oil hydrocarbon, such as a fixed gas, a gas oil, or a non-viscous neutral oil is chlorinated. A rubber material, such as crepe rubber, caoutchouc, or vulcanized rubber, is dissolved in a low boiling solvent such

as solvent naphtha. The chlorinated hydrocarbon is added and anhydrous aluminum chloride is introduced into the mixture of rubber, chlorinated hydrocarbon, and solvent. As the reaction 5 occurs, the temperature rises and hydrogen chloride is evolved. A solution results from which the stable products can be recovered by washing with lye and water and removing the solvent by distillation.

10 Several examples of the production of these products follow, from which the reaction conditions, the ratio of initial materials used in the aluminum chloride conversion step and the characteristics and effects of the products obtained 15 can be seen.

*Example III*

A gas oil obtained from an East Texas crude, having a gravity of 37° A. P. I., an initial boiling point of 478° F. and a final boiling point of 637° F. 20 is chlorinated by passing chlorine through it at a temperature below 200° F. The chlorination is discontinued when it is found that the oil contains about 14% chlorine by weight. A solvent naphtha with 200/350° F. boiling range, which 25 has been purified by treating with anhydrous aluminum chloride, is added to 500 grams of crepe rubber. The mixture of rubber and solvent is heated on a reflux condenser equipped with 30 a water trap until all the moisture has been driven off and is then allowed to cool. 1500 grams of the chlorinated gas oil are introduced into the rubber and solvent mixture and 200 grams of anhydrous aluminum chloride are slowly 35 added at room temperature under agitation. The temperature rises to about 120° F. and considerable volumes of hydrogen chloride are evolved. At the end of several hours the temperature is raised to about 190° F. and 220° F. 40 Steam is introduced into the resulting solution, vaporizing part of the solvent. When about half of the solvent has been distilled, the distillation is discontinued and the residual liquid is separated from the sludge. The liquid is washed with a lye solution, till neutral, and subjected to 45 distillation. A residual product is obtained having a high viscosity and the appearance of a lubricating oil. A blend of 2% by weight of the product with a lubricating oil is prepared. The tests on the original oil and the blend follow:

tation. The sludge is then allowed to settle and the naphtha solution is withdrawn for purification and redistillation as shown above. A residual oil is obtained showing the following inspection.

|                              |           |
|------------------------------|-----------|
| Gravity, °A. P. I.           | 23        |
| Saybolt viscosity at 100° F. | 3600 sec. |
| Saybolt viscosity at 210° F. | 165 sec.  |

A blend is prepared using two parts by weight of the synthetic oil and 100 parts by weight of a lubricating oil. The tests of the original lubricating oil and of the blend are shown below:

|                              | Original oil | Blend    | 15 |
|------------------------------|--------------|----------|----|
| Gravity, °A. P. I.           | 29.6         | 29.5     |    |
| Flash point                  | 420° F.      | 420° F.  |    |
| Saybolt viscosity at 100° F. | 187 sec.     | 196 sec. |    |
| Saybolt viscosity at 210° F. | 47 sec.      | 48 sec.  |    |
| Pour-point                   | +20° F.      | -5° F.   |    |
| Color, A. S. T. M.           | 3½           | 4½       | 20 |

*Example V*

30 litres of solvent naphtha having a boiling range of 200 to 350° F. are heated to about 110° F. During agitation, 2000 grams of crepe rubber are introduced. At the end of three hours the temperature is raised sufficiently to remove all the moisture by distilling off part of the solvent naphtha. 3000 grams of ethylene dichloride are 30 added to the resulting mixture, which has been cooled. At room temperature 450 grams of anhydrous aluminum chloride are slowly added. Under good agitation the temperature rises to about 100° F. and at the end of several hours 35 the temperature is raised to 190° F. Considerable volumes of hydrogen chloride are formed. After an additional two hours the mixture is cooled and allowed to settle.

The clear naphtha solution is withdrawn from the sludge. It is treated with a lye solution and water and subjected to distillation. A residual product is obtained having a clear red color and showing the following inspection:

|                              |           |
|------------------------------|-----------|
| Gravity, °A. P. I.           | 21        |
| Saybolt viscosity at 100° F. | 1350 sec. |
| Saybolt viscosity at 210° F. | 117 sec.  |
| Color, A. S. T. M.           | 3         |

A blend is prepared consisting of two parts by weight of the above oil and 100 parts by weight of a lubricating oil. The tests of the original lubricating oil and the blend are shown below:

|                              | Original oil | Blend    | 55 |
|------------------------------|--------------|----------|----|
| Gravity, °A. P. I.           | 29.7         | 29.6     |    |
| Flash                        | 420° F.      | 420° F.  |    |
| Saybolt viscosity at 100° F. | 192 sec.     | 206 sec. |    |
| Saybolt viscosity at 210° F. | 47 sec.      | 49 sec.  |    |
| Pour-point                   | +20° F.      | -5° F.   |    |
| Color, A. S. T. M.           | 3½           | 3½       | 60 |

An additional blend is made consisting of three parts by weight of the product prepared above and 100 parts by weight of a heavy lubricating oil. The tests of the heavy lubricating oil and of the blend follow:

|                              | Original oil | Blend     | 70 |
|------------------------------|--------------|-----------|----|
| Gravity, °A. P. I.           | 26.0         | 25.7      |    |
| Flash                        | 525° F.      | 540° F.   |    |
| Saybolt viscosity at 100° F. | 2288 sec.    | 2405 sec. |    |
| Saybolt viscosity at 210° F. | 148 sec.     | 155 sec.  |    |
| Pour-point                   | +25° F.      | +10° F.   |    |
| Color, A. S. T. M.           | 7½           | 7½        | 75 |

Additional 20 litres of solvent naphtha are added to the sludge left in the reaction kettle. Under agitation the mixture is heated to about 160° F. introducing 1 litre of water. The products are then allowed to cool and to settle. A clear naphtha solution is withdrawn and is washed with lye and water, whereafter the solution is subjected to distillation. A residual product is obtained. The product is blended with 10 equal parts of a lubricating oil showing the inspection of the original oil below. The tests of the blend are shown below:

|                                 |            |
|---------------------------------|------------|
| Gravity, °A. P. I.              | 19         |
| Saybolt viscosity at 100° F.    | 11000 sec. |
| 15 Saybolt viscosity at 210° F. | 346 sec.   |
| Pour-point                      | 15/20° F.  |
| Color, A. S. T. M.              | 5          |

A blend is prepared consisting of two parts by 20 weight of this blend, and 100 parts by weight of a lubricating oil. The inspections of the original lubricating oil and of the final blend follow:

|                              | Original oil | Blend    |
|------------------------------|--------------|----------|
| 25 Gravity, °A. P. I.        | 29.6         | 29.3     |
| Flash                        | 420° F.      | 425° F.  |
| Saybolt viscosity at 100° F. | 187 sec.     | 223 sec. |
| Saybolt viscosity at 210° F. | 47 sec.      | 52 sec.  |
| Pour-point                   | +20° F.      | -10° F.  |
| 30 Color, A. S. T. M.        | 3 1/4        | 3 3/4    |

I claim:

1. An improved lubricant comprising a blend of a major proportion of a wax-containing viscous hydrocarbon oil and a minor proportion of products obtained by dissolving rubber in a low boiling mineral oil fraction, adding anhydrous aluminum chloride, and effecting a conversion of the rubber with the aid of heat.
- 40 2. An improved lubricant comprising a blend of a major proportion of a wax-containing viscous hydrocarbon oil and a minor proportion of products obtained by acting upon rubber, while dissolved in a low boiling mineral oil fraction and in the presence of chlorinated hydrocarbons, with anhydrous aluminum chloride under temperature conditions effective to provide conversion products having pour point lowering properties.
- 45 3. An improved lubricant containing in major proportion a wax-containing viscous hydrocarbon oil and also containing, in minor proportion from about 0.05% to about 5.0% based on the weight of said oil, products derived from the conversion of a rubber material by the action of anhydrous aluminum chloride with the aid of heat under conditions effective to impart to said products pour point lowering properties, said lubricant having a pour point on the Fahrenheit scale lower than that of said oil by from about fifteen to about thirty-five degrees.
- 50 4. An improved lubricant having as a major constituent a wax-containing viscous hydrocarbon oil and containing, in relatively minor proportion based on the amount of said oil, products obtained by acting upon a rubber material, while in a dissolved phase, with anhydrous aluminum chloride under conditions effective to produce conversion products of rubber having pour point lowering properties.
- 55 5. An improved lubricant having as a major constituent a wax-containing viscous hydrocarbon oil and containing, in relatively minor proportion based on the amount of said oil, an anhydrous aluminum chloride conversion product

of rubber characterized by its effectiveness in substantially lowering the pour point of said oil.

6. An improved lubricant having as a major constituent a wax-containing viscous hydrocarbon oil and containing aluminum chloride conversion products of rubber capable of lowering the pour point of said hydrocarbon oil, said products being present in proportions of from about 0.05% to about 5.0% by weight based upon the amount of said hydrocarbon oil.

7. The method of preparing lubricants having as a major constituent a wax-containing viscous hydrocarbon oil, said lubricant having a pour point substantially lower than that of said oil, which comprises blending with said oil a minor proportion of products obtained by dissolving rubber in a low boiling mineral oil fraction, adding anhydrous aluminum chloride, and effecting a conversion of the rubber with the aid of heat.

8. The method of preparing lubricants having as a major constituent a wax-containing viscous hydrocarbon oil, said lubricant having a pour point substantially lower than that of said oil, which comprises blending with said oil a minor proportion of products obtained by acting upon a rubber material, while in a dissolved phase, with anhydrous aluminum chloride, and heating to effect a conversion of rubber to products characterized by a pour point lowering effect upon wax-containing hydrocarbon oils.

9. The method of preparing lubricants having as a major constituent a wax-containing viscous hydrocarbon oil, said lubricant having a pour point substantially lower than that of said oil, which comprises blending with said oil a minor proportion of products obtained by the anhydrous aluminum chloride conversion of a rubber material under conditions effective to produce conversion products characterized by a pour point lowering effect upon wax-containing hydrocarbon oils.

10. An improved lubricant having as a major constituent a wax-containing viscous hydrocarbon oil and containing, in relatively minor proportion based upon the amount of said oil, products obtained by acting upon a rubber material, while in a dissolved phase and in the presence of chlorinated hydrocarbons, with anhydrous aluminum chloride under conditions effective to produce conversion products having pour point lowering properties.

11. An improved lubricant having as a major constituent a wax-containing viscous hydrocarbon oil and containing, in relatively minor proportion based upon the amount of said oil, anhydrous aluminum chloride conversion products of rubber and chlorinated hydrocarbons characterized by effectiveness in substantially lowering the pour point of said oil.

12. The method of preparing lubricants having as a major constituent a wax-containing viscous hydrocarbon oil, said lubricant having a pour point substantially lower than that of said oil, which comprises blending with said oil a minor proportion of products obtained by acting upon a rubber material while in a dissolved phase and in the presence of chlorinated hydrocarbons, with anhydrous aluminum chloride, and heating to effect a conversion to products characterized by a pour point lowering effect upon wax-containing hydrocarbon oils.

13. The method of preparing lubricants having as a major constituent a wax-containing viscous hydrocarbon oil, said lubricant having a pour

5 point substantially lower than that of said oil, which comprises blending with said oil a minor proportion of products obtained by the anhydrous aluminum chloride conversion of rubber and chlorinated hydrocarbons under conditions effective to produce conversion products characterized by a pour point lowering effect upon wax-containing hydrocarbon oils.

14. An improved lubricant comprising a blend

of a major proportion of a wax-containing viscous hydrocarbon oil and a minor proportion of a product obtained by the conversion of rubber in the presence of a catalyst of the type exemplified by aluminum chloride, said product being characterized by its effectiveness in substantially lowering the pour point of said oil.

ERICH M. STEFFEN.

CERTIFICATE OF CORRECTION.

Patent No: 2,142,219.

January 3, 1939.

ERICH M. STEFFEN.

It is hereby certified that error appears in the printed specification of the above numbered patent requiring correction as follows: Page 1, second column, line 40, for the word "as" read at; page 2, second column, line 41, for "isomerization" read polymerization; and that the said Letters Patent should be read with this correction therein that the same may conform to the record of the case in the Patent Office.

Signed and sealed this 21st day of February, A. D. 1939.

Henry Van Arsdale.  
Acting Commissioner of Patents.

(Seal)

5 point substantially lower than that of said oil, which comprises blending with said oil a minor proportion of products obtained by the anhydrous aluminum chloride conversion of rubber and chlorinated hydrocarbons under conditions effective to produce conversion products characterized by a pour point lowering effect upon wax-containing hydrocarbon oils.

14. An improved lubricant comprising a blend

of a major proportion of a wax-containing viscous hydrocarbon oil and a minor proportion of a product obtained by the conversion of rubber in the presence of a catalyst of the type exemplified by aluminum chloride, said product being characterized by its effectiveness in substantially lowering the pour point of said oil.

ERICH M. STEFFEN.

CERTIFICATE OF CORRECTION.

Patent No: 2,142,219.

January 3, 1939.

ERICH M. STEFFEN.

It is hereby certified that error appears in the printed specification of the above numbered patent requiring correction as follows: Page 1, second column, line 40, for the word "as" read at; page 2, second column, line 41, for "isomerization" read polymerization; and that the said Letters Patent should be read with this correction therein that the same may conform to the record of the case in the Patent Office.

Signed and sealed this 21st day of February, A. D. 1939.

Henry Van Arsdale.  
Acting Commissioner of Patents.

(Seal)